# EUROPEAN PATENT SPECIFICATION

(11) **EP 0 018 777 B1**
(45) Date of publication and mention of the grant of the patent: **05.10.1983**
(21) Application number: 80301324.2
(22) Date of filing: 24.04.1980
(51) Int. Cl.: C10G 65/12, C10G 47/16

(54) **Catalytic upgrading of refractory hydrocarbon stocks**
Katalytische Aufbereitung schwerzubehandelnder Kohlenwasserstoffe
Amélioration catalytique de charges réfractaires d'hydrocarbures

(30) Priority: 02.05.1979 US 35153
(43) Date of publication of application: 12.11.1980
(73) Proprietor: MOBIL OIL CORPORATION, New York New York 10017 (US)
(72) Inventor: Gorring, Robert Lee, Washington Crossing Pennsylvania (US); Smith, Robert Lloyd, Hopewell Jersey (US)
(74) Representative: West, Alan Harry

## Description

This invention relates to catalytic upgrading of refractory hydrocarbon charge stocks, such as, for example, a coker gas oil or catalytic cracking cycle stock, in a dual bed hydrotreating/hydrocracking cascade system.

Present refinery practice in upgrading coker gas oil generally involves hydroprocessing to remove hetero-atoms, followed by fluid catalytic cracking or high pressure hydrocracking in a two step operation. Such processes have entailed high equipment costs associated with a two step operation. For example, GB Patent 1,191,471 describes a process for hydrocracking high boiling hydrocarbons to lower boiling hydrocarbons in a two stage hydrofining/hydrocracking procedure using pressures of 2860 to 27,600 kPa and 2860 to 20,800 kPa, respectively. Thus, catalytic cracking of even hydroprocessed material requires high severity operation causing excessive coke formation, leading to reduced catalyst life. The necessity to use high pressure has placed an additional economic burden on the overall process.

An improved process described in U.S. Patent 3,617,486 involves hydrofining a heavy hydrocarbon feed, hydrocracking the effluent and upgrading a 177-221 °C cut by 'hydrocrackfining' under low severity conditions. However, that process involves the use of fractionating and hydrocrackfining stages over and above those for the conventional hydrofining and hydrocracking, which generaly operate at about 3550-20,800 kPa.

U.S. Patent No. 3,957,621 discloses a process for producing alkyl aromatics, particularly parazylene, by hydrocracking over a ZSM-5 catalyst in combination with a hydrogenation/ dehydrogenation component a hydrocarbon charge containing aromatic hydrocarbons including benzene and C_{µ} alkyl aromatics and aliphatic hydrocarbons. The charge is rich in the aromatic hydrocarbons and lean in aliphatic hydrocarbons boiling above 220°F (104°C) by reason of conversion under severe conditions which comprise subjecting the charge to distillation such that at least a portion of the benzene content of the charge is separated as vapor from an alkyl aromatic fraction which contains a major portion of the C, aromatics in the charge and which is subjected to the subsequent hydrocracking process.

In accordance with the present invention, there has been discovered a dual bed hydrotreating/ hydrocracking cascade process for effectively upgrading refractory hydrocarbon stocks characterized by a bromine number greater than 10 and an aromatics content of at least 40 weight percent; such as coker gas oil and catalytic cracking cycle stock which process can be carried out at substantially lower pressures than those heretofore employed in the aforenoted two stage high pressure process.

The present process has been found to provide unexpectedly good yields and selectivity for the conversion of the above characterized refractory hydrocarbon feed to yield useful products including gasoline of high octane number, kerosene of low freeze point. Diesel or home heating fuel low in pour point and sulfur, and low sulfur distillate suitable for use as a catalytic cracking charge stock.

The refractory hydrocarbon feed, contemplated for upgrading in accordance with the present process contains at least about 40 and generally between about 40 and about 70 weight percent aromatics and has a Bromine No. in excess of about 10 and usually in the approximate range of 10 to 60. Exemplary of such feeds are low hydrogen refractory materials, such as catalytic cracking cycle stocks and coker gas oils, which are mostly poly-aromatic in structure and may contain appreciable amounts of sulfur, capable of being effectively removed in accordance with the present process.

The dual catalyst bed cascade process of this invention is conducted at a pressure within the approximate range of 790 to 12,512 kPa (100 to 1800 psig) and preferably between about 3549 and about 10443 kPa (500 and about 1500 psig). The temperature is generally within the approximate range of 288°C to 510°C (550°F to 950°F), with an increasing temperature gradient, as the feed passes initially through the bed of hydrotreating catalyst and thereafter through the bed of hydrocracking catalyst. Suitably, the temperature in the hydrotreating catalyst bed will be within the approximate range of 288°C to 454°C (500°F to 850°F) and in the hydrocracking catalyst bed within the approximate range of 343°C to 510°C (650°F to 950°F). The feed is conducted through the catalyst beds at an overall space velocity between about 0.1 and about 5 and preferably between about 0.2 and about 2, along with hydrogen initially present in the hydrotreating zone in an amount between about 180 and 1800 normal liters hydrogen per liter of feed, corresponding to a ratio of between about 2.4 and about 24 moles of hydrogen per mole of hydrocarbon and thereafter present in the hydrocracking zone in an amount between about 2 and about 23 moles of hydrogen per mole of charge to said hydrocracking zone.

The hydrotreating catalysts employed are generally metals or metal oxides of Group VIB and/or Group VIII deposited on a solid porous support such as silica and/or metal oxides such as alumina, titania, zirconia or mixtures thereof. Representative Group VIB include molybdenum, chromium and tungsten and Group VIII metals include nickel, cobalt, palladium and platinum. These metal components are deposited, in the form of metals or metal oxides, on the indicated supports in amounts generally between about 0.1 and about 20 weight percent.

Initial hydrotreating of the refractory hydrocarbon feed serves to convert sulfur and nitrogen derivatives of hydrocarbon to hydrogen sulfide and ammonia while depositing metal contaminant from hydrodecomposition of any ₒᵣganometal compounds. The entire effluent from the hydrotreating zone containing hydrogen, hydrocarbons, hydrogen sulfide and ammonia is passed to a hydrocracking zone over catalyst containing a crystalline aluminosilicate zeolite, characterized by a silica/alumina ratio greater than 12 and a constraint index, as hereinafter defined, in the approximate range of 1 to 12, such as, for example, zeolite ZSM-5 and a metal having activity to catalyze hydrogenation/dehydrogenation reactions. Representative of the latter metals are those of Groups VIII and other metals commonly referred to as transition metals.

Thus, the process, of this invention provides a dual bed system for upgrading a nitrogen and sulfur-containing hydrocarbon charge by contacting a stream of such charge initially in a hydrotreating zone containing a hydrotreating catalyst under the aforenoted conditions and thereafter passing the entire effluent from the hydrotreating zone to a hydrocracking zone containing a particularly defined crystalline aluminosilicate zeolite-containing hydrocracking catalyst under the above specified conditions of reaction. The latter zeolite-containing catalyst would appear to have the unique ability to bring pressure requirements for the hydrocracking zone to within the range of pressure employed in the hydrotreating zone, i.e. permit use of lower pressures in the hydrocracking zone over those previously employed. Moreover, the ability of the present process to convert the above stocks, such as coker gas oil to high octane gasoline, which can be directly blended to pool octane gasoline without the need for reforming is a significant feature differentiating the present operation from previous high pressure hydrocracking systems which produce low octane naphtha.

The crystalline aluminosilicate zeolites utilized herein are members of a novel class of zeolites that exhibits unusual properties.

Briefly, the preferred type zeolites useful in this invention possess, in combination: a silica to alumina mole ratio of at least about 12; a dried crystal density of not less than about 1.6 grams per cubic centimeter and a constraint index of about 1 to about 12. Crystal density constraint index and the measurement thereof are described in U.S. 4,118,431.

An important characteristic of the crystal structure of this class of zeolites is that is provides constrained access to and egress from the intracrystalline free space by virtue of having an effective pore size intermediate between the small pore Linde A and the large pore Linde X.

Although zeolites with a silica to alumina ratio of at least 12 are useful, it is preferred to use zeolites having high ratio of at least about 30. Such zeolites, after activation, acquire an intracrystalline sorption capacity for normal hexane which is greater -than -that for water, i.e., they exhibit "hydrophobic" properties.

When synthesized in the alkali metal form, the zeolite is conveniently converted to the hydrogen form, generally by intermediate formation of the ammonium form as a result of ammonium ion exchange and calcination of ammonium form to yield the hydrogen form. In addition to the hydrogen form, other forms of the zeolite wherein the original alkali metal has been reduced to less than about 1.5 percent by weight may be used. Thus, the original alkali metal of the zeolite may be replaced by ion exchange with other suitable ions of groups IB to VIII of the Periodic Table, including, by way of example, nickel, copper, zinc, palladium, calcium or rare earth metals.

Generally, however, the zeolite either directly or via initial ammonium exchange followed by calcination, is preferably hydrogen exchanged such that a predominate proportion of its exchangeable cations are hydrogen ions. In general, it is contemplated that more than 50 percent and preferably more than 75 percent of the cationic sites of the crystalline aluminosilicate zeolite will be occupied by hydrogen ions.

The class of zeolites defined herein is exemplified by ZSM-5, ZSM-11, ZSM-12, ZSM-23, ZSM-35 and ZSM-38, defined respectively by the X-ray diffraction data presented in U.S. 3,702,886, U.S. 3,709,979, U.S. 3,832,449, U.S. 4,076,842, U.S. 4,016,245 and U.S. 4.046,859. The preferred zeolite is ZSM-5.

In practicing the desired conversion process, it may be desirable to incorporate the above described crystalline aluminosilicate zeolite in another material resistant to the temperature and other conditions employed in the process. Such matrix materials include synthetic or naturally occurring substances as well as inorganic materials such as clay, silica and/or metal oxides.

The above zeolite, either as such or after compositing with a matrix, is combined with a minor amount, generally between about 0.1 and about 20 weight percent of a metal having hydrogenation/dehydrogenation promotion properties. Preferred metals are those of Groups VIII of the Periodic Table. Palladium is highly effective, as are the other Group VIII noble metals platinum, iridium, osmium, ruthenium and rhodium. Nickel, cobalt, etc. are effective. Other metals, particularly those called transition metals may be employed. The metal may be used alone or in combination, e.g., palladium and zinc. The metals may be incorporated in the finished catalyst by any of the techniques well known in the art such as base exchange, impregnation and the like.

Conditions for effective hydrotreating are well known and need no detailed review except to note that cascading the hydrotreater effluent to the second stage requires that sufficient hydrogen be supplied with charge to the hydrotreater zone in order that requirements of both stages shall be satisfied. Pressure in the system described herein will be the same for the hydrotreating and hydrocracking zones and generally within the approximate range of 790 to 12512 kPa (100 to 1800 psig) and preferably between about 3549 and about 10443 kPa (500 and about 1500 psig). Generally, it will be found desirable to employ higher temperature in the second than in the first stage to achieve high conversion to lower boiling products in the second stage. this is accomplished by inter-stage heating. Space velocities for the two stages are adjusted by sizes of the catalyst beds.

The following examples will serve to illustrate the process of the invention without limiting the same:

### Example 1

A coker heavy gas oil was processed, along with hydrogen, in a system made up of an initial bed of hydrotreating catalyst and second bed of hydrocracking catalyst.

The charge stock has the following properties:

Operating conditions included a pressure of 6996 kPa (1000 psig), a hydrogenating catalyst bed temperature of 371-389°C (700-732°F), a hydrocracking bed temperature of 424-464°C (796-868°F), hydrogen in the amount of 450 normal liters of hydrogen per liter (2500 standard cubic feet of hydrogen per barrel) of charge and an overall space velocity of 0.3-0.5.

The hydrotreating catalyst was in the form of an extrudate having a surface area of 129 m^{Z}/gram and containing, expressed as weight percent oxides, the following metals:

Effluent from the hydrotreating zone was passed directly without interstage separation to a hydrocracking zone containing catalyst. The hydrocracking catalyst was HZSM-5 containing 0.5 weight percent palladium and 0.6 weight percent zinc. This catalyst, having a surface area of 315 m²/gram, was prepared by ion-exchanging HZSM-5 with aqueous Zn(N0₃)₂, followed by water washing and impregnation of the wet cake with aqueous palladium tetramine nitrate, after which, the composite was dried and calcined at 538°C (1000°F). The resulting material was wet slurried with 35 weight percent Al₂O₃, extruded in the form of 1.6 mm (1/16") particles, dried and calcined in air at 538°C (1000°F).

The results obtained in runs extending from 6 to 41 days are set forth in the following Table:

It will be seen from the above tabulated data that the same show net conversion as high as 49% to 282°C (540°F-) and 44% to 216°C- (420°F-). The total yield of naphtha plus distillate C₄-454°C (850°F) was as much as 89%. Moreover, it will be seen that the catalyst exhibited good stability as evident from results obtained after an uninterrupted on-stream period of 41 days.

Separation of representative liquid products was effected by fluorescent indicator adsorption into volume percent aromatics, olefins and saturates. Results for the liquid products obtained in Run Nos. 1, 5, 6 and 7 of Table 1 are shown below.

The liquid yield from run 3 (identified in Table 1) was fractionated into products of appropriate boiling ranges having the properties set out in the following Table 3:

It will be evident from the foregoing that useful product fractions show a pool octane quality gasoline containing 31% aromatics (86 RON-Clear); a light gas oil suitable for diesel fuel or No. 2 fuel (.05% sulfur) and a heavier fraction with 0.3% sulfur useful as a cracking stock.

## Claims

1. A dual bed process for upgrading a refractory hydrocarbon feed selected from coker gas oil and catalytic cracking cycle stock having a Bromine No. greater than 10 and an aromatics content of at least 40 weight percent, which comprises contacting a stream of the refractory hydrocarbon feed intially in a hydrotreating zone containing a bed of hydrotreating catalyst under reaction conditions which include a pressure within the range of 790 to 12512 kPa, a temperature between 288°C and 454°C in the presence of between 2.4 and 24 moles of hydrogen/mole of refractory hydrocarbon feed; passing the entire effluent from the hydrotreating zone to a hydrocracking zone containing a bed of hydrocracking catalyst comprising a crystalline aluminosilicate zeolite having a silica to alumina ratio of at least 12 and a constraint index within the range of 1 to 12 in combination with a metal component exhibiting hydrogenation/dehydrogenation activity under reaction conditions which include a pressure within the above stated range, a hydrogen concentration between 2 and 23 moles of hydrogen per mole of charge to the hydrocracking zone and a temperature between 343°C and 510°C.

2. The process of Claim 1 characterized in that the refractory hydrocarbon feed contains between 40 and 70 weight percent or aromatics and has a Bromine No. in the range of 10 to 60.

3. The process of any preceding claim characterized in that the refractory hydrocarbon feed is a catalytic cracking cycle stock.

4. The process of any preceding claim characterized in that the refractory hyodrcarbon feed is coker gas oil.

5. The process of any preceding claim characterized in that the zeolite is ZSM-5.

6. The process of any preceding claim characterized in that the metal component is palladium, zinc or a combination of palladium and zinc.

## Revendications

1. Un procédé à lit double pour le raffinage d'une charge d'hydrocarbure réfractaire choisie parmi le gas-oil de cokerie et la charge de recyclage de craquage catalytique ayant un indice de brome supérieur à 10 et une teneur en aromatiques d'au moins 40 % en poids, qui comprend la mise en contact d'un courant de la charge d'hydrocarbure réfractaire initialement dans une zone d'hydrotraitement contenant un lit de catalyseur d'hydro-traitement dans des conditions de réaction comprenant une pression dans la gamme de 790 à 12 512 kPa, une température entre 288 et 454°C, en présence de 2,4 à 24 moles d'hydrogène/mole de charge d'hydrocarbure réfractaire; le passage de la totalité de l'effluent de la zone d'hydro-traitement à une zone d'hydrocraquage contenant un lit de catalyseur d'hydrocraquage comprenant un alumino-silicate cristallin du type zéolite ayant un rapport silice/alumine d'au moins 12 et un indice de contrainte dans la gamme de 1 à 12 en combinaison avec un composant métallique présentant une activité d'hydrogénation/déhydrogénation dans des conditions de réaction qui comprennent une pression comprise dans la gamme indiquée ci-dessus, une concentration d'hydrogène entre 2 et 23 moles d'hydrogène par mole de la charge introduite dans la zone d'hydrocraquage et une température comprise entre 343 et 510°C.

2. Le procédé selon la revendication 1, caractérisé en ce que la charge d'hydrocarbure réfractaire contient entre 40 et 70 % en poids d'aromatiques et possède un indice de brome dans l'intervalle de 10 à 60.

3. Le prcédé selon l'une quelconque des revendications précédentes, caractérisé en ce que la charge d'hydrocarbure réfractaire est une charge de recyclage de craquage catalytique.

4. Le procédé selon l'une quelconque des revendications précédentes, caractérisé en ce que la charge d'hydrocarbure réfractaire est du gas-oil de cokerie.

5. Le procédé selon l'une quelconque des revendications précédentes, caractérisé en ce que la zéolite est la ZSM-5.

6. Le procédé selon l'une quelconque des revendications précédentes, caractérisé en ce que le composant métallique est le palladium, le zinc ou une combinaison de palladium et de zinc.

## Patentansprüche

1. Ein Doppelbett-Verfahren zur Qualitätsverbesserung eines schwer aufbereitbaren Kohlenwasserstoff-Rohstoffs, der aus Cokergasöl und einem Umlauföl vom katalytischen Cracken mit einer Bromzahl von mehr als 10 und einem Aromatengehalt von wenigstens 40 Gewichtsprozent ausgewählt ist, bei dem eine Strom des schwer aufbereitbaren Kohlenwasserstoff-Rohstoffs zuerst in einer Wasserstoffbehandlungs-Zone, die ein Bett eines Wasserstoffbehandlungs-Katalysators enthält, unter Reaktionsbedingungen, die einen Druck im Bereich von 790 bis 12 512 kPa, eine Temperatur zwischen 288°C und 454°C umfassen, in Gegenwart von zwischen 2,4 und 24 Mol Wasserstoff/Mol des schwer aufbereitbaren Kohlenwasserstoff-Rohstoffs am Kontakt umgesetzt wird; bei dem dann das Gesamte abströmende Produkt aus der Wasserstoffbehandlungs-Zone in eine Hydrocrack-Zone weitergeleitet wird, die ein Bett eines Hydrocrack-Katalysators enthält, der einen kristallinen Alumosilikat-Zeolith mit einem Verhältnis von Siliciumoxid zu Aluminiumoxid von wenigstens 12 und einem Grenzwertindex (constraint index) im Bereich von 1 bis 12 in Kombination mit einem Metallbestandteil enthält, der eine Hydrier/Dehydrier-Wirkung unter den Reaktionsbedingungen aufweist, die einen Druck im oben angegebenen Bereich, eine Wasserstoffkonzentration zwischen 2 und 23 Mol Wasserstoff pro Mol des der Hydrocrack-Zone zugeführten Materials und eine Temperatur zwischen 343°C und 510°C umfassen.

2. Verfahren nach Anspruch 1, dadurch gekennzeichnet, daß der schwer aufbereitbare Kohlenwasserstoff-Rohstoff zwischen 40 und 70 Gew.-% Aromaten enthält und eine Bromzahl im Bereich von 10 bis 60 aufweist.

3. Verfahren nach einem beliebigen der vorangehenden Ansprüche, dadurch gekennzeichnet, daß der schwer aufbereitbare Kohlenwasserstoff-Rohstoff ein Umlauföl vom Katalytischen Cracken ist.

4. Verfahren nach einem beliebigen der vorangehenden Ansprüche, dadurch gekennzeichnet, daß der schwer aufbereitbare Kohlenwasserstoff-Rohstoff Cokergasöl ist.

5. Verfahren nach einem beliebigen der vorangehenden Ansprüche, dadurch gekennzeichnet, daß der Zeolith ZSM-5 ist.

6. Verfahren nach einem beliebigen der vorangehenden Ansprüche, dadurch gekennzeichnet, daß der Metallbestandteil Palladium, Zink oder eine Kombination aus Palladium und Zink ist.
